

## UNITED STATES PATENT OFFICE

2,160,293

## LUBRICANT

Bernard H. Shoemaker and Clarence M. Loane,  
Hammond, Ind., assignors to Standard Oil Company,  
Chicago, Ill., a corporation of Indiana

No Drawing. Application December 5, 1936,  
Serial No. 114,434

## 10 Claims.

(Cl. 87—9)

This invention relates to lubricants and, in particular, to addition agents imparting improved properties to lubricants.

This invention has particular utility in improving the lubricating properties of lubricating oils and/or in preventing or inhibiting the corrosion of "hard metal" alloy bearings such as copper-lead, cadmium-nickel and cadmium-silver bearings which, to a large extent, have replaced soft metal bearings, such as Babbitt metal, in the trend toward internal combustion engines having high compression ratios and increased acceleration and increased speed characteristics. The use of the "hard metal" bearings has created lubricating and corrosion problems, particularly in connection with highly refined oils, some of which may be very corrosive to bearings of the hard metal type.

As used herein "highly refined" lubricating oil means viscous oils which have a minimum viscosity of S. A. E. 10 oils and oils having higher viscosities, and which have been subjected to such refining processes that the paraffinicity of the oil is markedly increased. It has been found that "highly refined" lubricating oils cause corrosion to alloy bearings of the hard metal type such as cadmium-silver alloy bearings to the extent of about 5 mg/cm.<sup>2</sup> and even greater when such bearings are submerged for 25 hours or less in an air agitated oil which has been preoxidized at about 340° F. for 25 to 50 hours. The motor oils may be "highly refined" lubricating oils as such or mixtures of highly refined lubricating oils with less highly refined lubricating oils, or stated in another way, mixtures of corrosive oils and non-corrosive oils, examples of the latter being lubricating oil fractions from Winkler crude or crudes of the Winkler type.

We have found that corrosion of hard metal alloy bearings can be inhibited and highly desirable properties can be imparted to lubricating oils by adding thereto up to 5%, but preferably 0.05% to 0.75%, of a poly membered heterocyclic compound having the general formula A—R in which A represents a heterocyclic radical selected from the group consisting of azoles containing only nitrogen and carbon in the ring, azines containing only nitrogen and carbon in the ring, pyrroles and thiophenes, and R represents hydrogen or a substituted radical or radicals, such as alkyl or aryl or aralkyl or alkoxy or mercapto or amino or substituted amino or halogen and/or mixtures thereof.

The term azole as used herein comprises the penta heterocyclic compounds having two, three

or four nitrogen atoms only in the ring such as: pyrazole (1,2-diazole or pyrro (a) monazole), glyoxaline or imidazol (1,3-diazole), 1,2,4-triazole (pyrro (ab<sub>1</sub>) diazole), 1,3,4-triazole (pyrro (bb<sub>1</sub>) diazole), 1,2,3-triazole (pyrro (ab) diazole), 1,2,5-triazole (pyrro (aa<sub>1</sub>) diazole), 1,2,3,4-tetrazole (pyrro (abb<sub>1</sub>) triazole), 1,2,3,5-tetrazole (pyrro (aba<sub>1</sub>) triazole); and the hereinbefore mentioned substituted derivatives in which the following numbering system is used:



Examples of the substituted derivatives of the above are: n-octyl pyrazoles, phenyl pyrazoles, phenyl dimethyl pyrazoles, di, tri and/or tetra methyl pyrazoles, chlor pyrazoles, amino pyrazoles, amino trimethyl pyrazoles, phenyl ethoxy pyrazoles, methyl glyoxalines, phenyl glyoxalines, 4-methyl phenyl glyoxalines, chloro methyl glyoxalines, 4,5-diphenyl glyoxaline-2-mercaptan, 5-amino ethyl glyoxaline, phenyl 1,2,5-triazoles, phenyl methyl 1,2,5-triazoles, amino-1,2,5-triazoles, phenyl 1,2,3-triazoles, phenyl ethoxy 1,2,3-triazoles, phenyl amino 1,2,3-triazoles, amino methyl 1,2,3-triazoles, methyl 1,2,4-triazoles, phenyl 1,3,4-triazoles, 1-phenyl 1,2,3,4-tetrazole, 1-methyl 1,2,3,4-tetrazole, 1-phenyl-2-methyl 1,2,3,4-tetrazole, mercapto tetrazoles, amino tetrazoles.

The term azine as used herein comprises the hexa-heterocyclic compounds having two or more nitrogen atoms only in the ring such as: pyridazine (1,2-diazine or orthodiazine), pyrimidine (1,3-diazine or metadiazine), pyrazine (1,4-diazine or paradiazine), as-triazine (1,2,4-triazine), s-triazine (1,3,5-triazine or cyanidine), v-triazine (1,2,3-triazine), s-tetrazine (1,2,4,5-tetrazine), v-tetrazine (1,2,3,4-tetrazine); and the hereinbefore mentioned substituted derivatives in which the following numbering system is used:



Examples of derivatives of the above named compounds are: methyl pyridazines, phenyl pyridazines, methyl phenyl pyridazines, methyl pyrimidines, methyl ethyl pyrimidines, methyl phenyl pyrimidines, dimethyl amino pyrimidines, 55

- amino pyrimidines, chloro dimethyl pyrimidines, 2,4,5,6-tetra chloro pyrimidine, methyl pyrazines, diphenyl pyrazines, diphenyl methyl cyanides, diphenyl cyanides, triphenyl cyanides, trimethyl cyanides, tributoxy cyanides, chloro trimethyl cyanides, amino cyanides, diphenyl 1,2,3,4-tetrazine.

The term *pyrrole* as used herein, comprises the penta heterocyclic compounds having a 4-membered carbon chain united to a ring by a bivalent imino ( $\text{NH}=\text{}$ ) group (sometimes called the imine group) and the hereinbefore mentioned substituted derivatives thereof such as: methyl pyrroles, ethyl pyrroles, isoamyl pyrroles, phenyl pyrroles, methyl phenyl pyrroles.

The term *thiophenes* as used herein comprises the penta heterocyclic compounds having only sulfur and carbon in the ring of the general structural formula



and the hereinbefore mentioned substituted derivatives thereof, such as: lauryl thiophenes, di-cyclohexyl thiophenes, isopropyl thiophenes, hexyl thiophenes, phenyl thiophenes, diphenyl thiophenes, tetraphenyl thiophenes, methyl phenyl thiophenes, chlorothiophenes, diamyl 30 aminothiophenes, thiophthens (bithiophenes).

In addition to the hereinbefore mentioned types of compounds we may use other compounds closely related to the foregoing such as pyridine, quinoline, brucine, thienyls such as 35 dithienylmethane, thienyltriphenylmethane, and the like.

The effectiveness of these compounds as corrosion inhibitors is demonstrated by the following test in which the inhibitor was subjected to 40 conditions more severe than those encountered in the actual operation of internal combustion engines. In this test weighed cadmium-silver alloy bearings were placed in containers containing a highly refined oil with and without 45 the addition of the inhibitors and the oil air agitated and maintained at a temperature of about 341° F. At periodic intervals the bearings were removed from the oil baths, washed free of the oil and the loss in weight determined. 50 Before being replaced in the oil bath the bearings were polished bright, reweighed and again tested for predetermined periods. In this test the oil used was a motor oil refined to such an extent that a loss in weight of more than 5 55 mg/cm.<sup>2</sup> is obtained in 25 hours or less on a cadmium-silver alloy bearing submerged in the air agitated oil at about 341° F., which oil had been preoxidized for 25 to 50 hours at about 341° F.

60 In the table below are tabulated the results obtained in the above test using tributoxy cyanidine (1,3,5-triazine) as the inhibitor.

Loss in weight (mg/cm.<sup>2</sup>)

| 65 | Oil                              | Periods      |             |              |
|----|----------------------------------|--------------|-------------|--------------|
|    |                                  | 1st, 24 hrs. | 2nd, 6 hrs. | 3rd, 16 hrs. |
| 70 | Control                          | 3.59         | 5.06        | 20.5         |
|    | Control+0.2% tributoxy cyanidine | 0.24         | 0.00        | 0.11         |

The above data illustrates the high inhibiting power of compounds of the type hereinbefore 75 described.

Some of the hereinbefore named compounds may not be completely soluble in the lubricant in which case effective results may be obtained by suspending the inhibitor in the lubricant by means of a small amount of a peptizing agent such as aluminum naphthenate, aluminum stearate and the like.

We do not wish to limit ourselves to the specific embodiments of our invention herein described except as defined by the appended claims. 10

We claim:

1. A motor oil non-corrosive to hard metal alloy bearings having the corrosive susceptibility of alloys of the class consisting of cadmium-silver, cadmium-nickel, copper-lead alloys consisting of a mineral lubricating oil normally corrosive to said hard metal alloys and a small amount of a polymembered heterocyclic compound having the general formula A-R in which A represents a heterocyclic radical selected from the group consisting of azoles, containing only nitrogen and carbon in the ring, azines, containing only nitrogen and carbon in the ring, pyrroles and thiophenes and R is a substituent selected from the group consisting of hydrogen, an alkyl radical, an aryl radical, an aralkyl radical, an alkoxy radical, a mercapto radical, an amino radical, a substituted amino radical and a halogen, said polymembered heterocyclic compound being added in small but sufficient quantities to inhibit the corrosion of said hard metal alloy bearings. 20

2. A motor oil non-corrosive to hard metal alloy bearings having the corrosive susceptibility of alloys of the class consisting of cadmium-silver, cadmium-nickel and copper-lead alloys consisting of a mineral lubricating oil normally corrosive to said bearings and a polymembered heterocyclic compound having the general formula A-R in which A represents an azole containing only nitrogen and carbon in the ring and R is a substituent selected from the group consisting of hydrogen, an alkyl radical, an aryl radical, an aralkyl radical, an alkoxy radical, a mercapto radical, an amino radical, a substituted amino radical and a halogen, said polymembered heterocyclic compound being added in small but sufficient quantities to inhibit the corrosion of said hard metal alloy bearings. 35

3. A motor oil non-corrosive to hard metal alloy bearings having the corrosive susceptibility of alloys of the class consisting of cadmium-silver, cadmium-nickel and copper-lead alloys consisting of a mineral lubricating oil normally corrosive to said bearings and a polymembered heterocyclic compound having the general formula A-R in which A represents an azine containing only nitrogen and carbon in the ring and R is a substituent selected from the group consisting of hydrogen, an alkyl radical, an aryl radical, an aralkyl radical, an alkoxy radical, a mercapto radical, an amino radical, a substituted amino radical and a halogen, said polymembered heterocyclic compound being added in small but sufficient quantities to inhibit the corrosion of 40 said hard metal alloy bearings. 50

4. A motor oil non-corrosive to hard metal alloy bearings having the corrosive susceptibility of alloys of the class consisting of cadmium-silver, cadmium-nickel and copper-lead alloys consisting of a mineral lubricating oil normally corrosive to said bearings and a polymembered heterocyclic compound having the general formula A-R in which A represents a thiophene containing only nitrogen and carbon in the ring 75

and R is a substituent selected from the group consisting of hydrogen, an alkyl radical, an aryl radical, an aralkyl radical, an alkoxy radical, a mercapto radical, an amino radical, a substituted amino radical and a halogen, said polymembered heterocyclic compound being added in small but sufficient quantities to inhibit the corrosion of said hard metal alloy bearings.

5. A motor oil non-corrosive to hard metal alloy bearings having corrosive susceptibility of alloys of the class consisting of cadmium-silver, cadmium-nickel and copper-lead alloys consisting of a mineral lubricating oil normally corrosive to said bearings and tributoxy cyanidine, 5 said tributoxy cyanidine being used in small but sufficient quantities to inhibit the corrosion of said hard metal alloy bearings.

6. A motor oil non-corrosive to hard metal alloy bearings having corrosive susceptibility of alloys of the class consisting of cadmium-silver, cadmium-nickel and copper-lead alloys consisting of a mineral lubricating oil normally corrosive to said bearings and hexyl thiophene, said hexyl thiophene being used in small but sufficient quantities to inhibit the corrosion of said hard metal alloy bearings.

7. The method of preventing corrosion of bearing metal alloys having the corrosive susceptibility of alloys of the class consisting of cadmium-silver alloys, cadmium-nickel alloys, copper-lead alloys in the presence of highly refined lubricating oils in internal combustion engines which comprises adding to said lubricating oil from about 0.05% to about 5% of a polymembered heterocyclic compound having the general formula A-R in which A represents a heterocyclic radical selected from the group consisting of azoles containing only nitrogen and carbon in the ring, azines containing only nitrogen and carbon in the ring, pyrroles and thiophenes and R is a substituent selected from the group consisting of hydrogen, an alkyl radical, an aryl radical, an aralkyl radical, an alkoxy radical, a mercapto radical, an amino radical, a substituted amino radical and a halogen.

8. The method of preventing corrosion of bearing metal alloys having the corrosive susceptibility of alloys of the class consisting of cad-

mium-silver alloys, cadmium-nickel alloys, copper-lead alloys in the presence of highly refined lubricating oils in internal combustion engines which comprises adding from about 0.05% to about 5% of a polymembered heterocyclic compound having the general formula A-R in which A represents an azole containing only nitrogen and carbon in the ring and R is a substituent selected from the group consisting of hydrogen, an alkyl radical, an aryl radical, an aralkyl radical, an alkoxy radical, a mercapto radical, an amino radical, a substituted amino radical and a halogen.

9. The method of preventing corrosion of bearing metal alloys having the corrosive susceptibility of alloys of the class consisting of cadmium-silver alloys, cadmium-nickel alloys, and copper-lead alloys in the presence of highly refined lubricating oils in internal combustion engines which comprises adding to said lubricating oil from about 0.05% to about 5% of a polymembered heterocyclic compound having the general formula A-R in which A represents azines containing only nitrogen and carbon in the ring and in which R is a substituent selected from the group consisting of hydrogen, an alkyl radical, an aryl radical, an aralkyl radical, an alkoxy radical, a mercapto radical, an amino radical, a substituted amino radical and a halogen.

10. The method of preventing corrosion of bearing metal alloys having the corrosive susceptibility of alloys of the class consisting of cadmium-silver alloys, cadmium-nickel alloys and copper-lead alloys in the presence of highly refined lubricating oils in internal combustion engines which comprises adding to said lubricating oil from about 0.05% to about 5% of a polymembered heterocyclic compound having the general formula A-R in which A represents thiophenes and R is a substituent selected from the group consisting of hydrogen, an alkyl radical, an aryl radical, an aralkyl radical, an alkoxy radical, a mercapto radical, an amino radical, a substituted amino radical and a halogen.

BERNARD H. SHOEMAKER.  
CLARENCE M. LOANE.

CERTIFICATE OF CORRECTION.

Patent No. 2,160,293.

May 30, 1939.

BERNARD H. SHOEMAKER, ET AL.

It is hereby certified that error appears in the printed specification of the above numbered patent requiring correction as follows: Page 2, second column, line 46, claim 2, for "mino" read amino; and that the said Letters Patent should be read with this correction therein that the same may conform to the record of the case in the Patent Office.

Signed and sealed this 25th day of July, A. D. 1939.

(Seal)

Henry Van Arsdale,  
Acting Commissioner of Patents.